

Patented June 19, 1928.

1,674,166

# UNITED STATES PATENT OFFICE.

WILLIAM A. DOUGLASS, OF PENNS GROVE, NEW JERSEY, ASSIGNOR TO E. I. DU PONT DE NEMOURS & COMPANY, OF WILMINGTON, DELAWARE, A CORPORATION OF DELAWARE.

## PROCESS OF CONCENTRATING ORES AND MINERALS BY FLOTATION.

No. Drawing.

Application filed June 25, 1926. Serial No. 118,590.

This invention relates to the recovery of valuable ores and minerals by flotation and comprises more particularly the concentration of such ores and minerals by means of a 5 certain class of organic flotation agents.

I have discovered that flotation processes may be carried out very efficiently by the use of a very highly selective class of compounds, including alkyl thio urethanes and 10 their derivatives. This class of compounds is characterized by having the following general graphical formula:



15 in which R is any alkyl group and R<sup>1</sup> and R<sup>2</sup> represent hydrogen, or alkyl groups. These compounds are superior flotation 20 agents and are susceptible of wide application. They may be prepared with comparative ease and in most cases are readily soluble in alkaline solutions. This solubility permits the use of the flotation agents in solution and by adding a solution of the agent just prior to actual flotation, it is possible to dispense with pre-agitation of the ore pulp with the flotation reagent. However, even 25 when the reagents are not used in solution, it has been found that only a very brief pre-agitation with the ore pulp is required to obtain proper dispersion.

The following are given as examples of 30 some of the compounds which may be used in the present invention and conforming to the general structural formula disclosed:



40 and corresponding derivatives of the homologous series of alcohols, such as:



45 as well as the corresponding derivatives of the homologous series of aliphatic amines.

Flotation tests made with compounds of this type as the flotation reagent were carried out in the following manner: Five hundred grams of ore from the Utah Copper Co. were ground 5 minutes in a ball mill with 350 cc. of water and 2.2 grams of lime. The pulp from the ball mill was

transferred to a Janney laboratory flotation 55 machine and diluted to a total volume of about 900 cc. After one-half minute pre-agitation, .04 gram of pine oil and .025 gram of the flotation agent were added and the pre-agitation continued one minute 60 longer. The pulp was diluted to cause circulation, and froth was removed for 7 minutes, water being added as needed during the test. The results of this test were as follows:

|                        |            |
|------------------------|------------|
| Heads                  | 1.06% Cu.  |
| Concentrates (rougher) | 15.50% Cu. |
| Tailings               | 19% Cu.    |
| Recovery               | 83.2%      |

70 A test was made on ore from the Phelps-Dodge Corporation using the same general procedure as outlined above. The results are included in the following data:

|                       |                      |
|-----------------------|----------------------|
| Phenyl thio urethane  | .10 lb. per ton ore. |
| Lime                  | 2.4 lb. per ton ore. |
| Heads                 | 1.48% Cu.            |
| Concentrate (rougher) | 6.66% Cu.            |
| Tailings              | 21% Cu.              |
| Recovery              | 88.6%                |

75 When ore from the Phelps-Dodge Corporation was treated in the Callow cell and the new flotation compound dissolved in a sodium hydroxide solution prior to its addition to the cell the results obtained were practically the same as when the Janney machine was used.

On ore from the Anaconda Copper Mining Company the new flotation agents were found to give good results when only .02 lb. per ton of ore was used with an alkaline circuit.

When ore from the Inspiration Copper Company was treated in the Callow cell, a flotation agent of the type disclosed, added to the cell in sodium hydroxide solution gave 90 equally good results.

The new flotation agents have little frothing power and, therefore, it is generally necessary to use a suitable frothing agent, such as pine oil or a light creosote oil in conjunction with these compounds. The use of the frothing agent is not always necessary, 100 however, when certain of the present flotation agents are used, but it is usually advantageous to employ a frothing agent with the flotation reagent.

105 Although in illustrating my new process, reference has been made specifically to copper ore, and to various specific conditions of operation, it will be understood that the

present invention is not limited to specific substances or conditions but includes generally processes of recovering values from ores by flotation in which the flotation agents are compounds of the class described.

The invention is not limited to the specific examples and substances disclosed but may be modified in many respects without departing from the scope thereof.

10 I claim:

1. In the process of concentrating ores and minerals by flotation, the step which comprises subjecting the ore in the form of a pulp to a flotation operation in the presence 15 of a substance having the following general molecular formula:



20 where R represents any alkyl group, and R<sup>1</sup>

and R<sup>2</sup> represent hydrogen or alkyl groups.

2. In the process of concentrating ores and minerals by flotation the step which comprises subjecting the ore in the form of a pulp to a flotation operation in the presence 25 of an alkyl thio urethane.

3. In the process of concentrating ores and minerals by flotation, the step which comprises subjecting the ore in the form of a pulp to a flotation operation in the presence 30 of a substance having the following general molecular formula:



35 where R represents an alkyl group, R<sup>1</sup> represents an alkyl group and R<sup>2</sup> represents hydrogen.

40 In testimony whereof I affix my signature.

WILLIAM A. DOUGLASS.